# EUROPEAN PATENT SPECIFICATION

(11) **EP 3 677 700 B1**
(45) Date of publication and mention of the grant of the patent: **10.05.2023**
(21) Application number: 18851150.5
(22) Date of filing: 29.08.2018
(51) Int. Cl.: C22C 38/00, C21D 8/02, C22C 38/38, C22C 38/02, C22C 38/04, C22C 38/06

(54) **HIGH-MN STEEL AND PRODUCTION METHOD THEREFOR**
STAHL MIT HOHEM MN-GEHALT UND HERSTELLUNGSVERFAHREN DAFÜR
ACIER RICHE EN MN ET SON PROCÉDÉ DE PRODUCTION

(30) Priority: 01.09.2017 JP 2017168857
(43) Date of publication of application: 08.07.2020
(73) Proprietor: JFE Steel Corporation, Tokyo 100-0011 (JP)
(72) Inventor: IZUMI, Daichi, Tokyo 100-0011 (JP); UEDA, Keiji, Tokyo 100-0011 (JP); HASE, Kazukuni, Tokyo 100-0011 (JP); NAKASHIMA, Koichi, Tokyo 100-0011 (JP)
(74) Representative: Grünecker Patent- und Rechtsanwälte PartG mbB
(86) International application number: PCT/JP2018/032022
(87) International publication number: WO 2019/044928

(56) References cited:
- EP-A1- 3 078 447
- JP-A- S56 258
- JP-A- S5 867 824
- JP-A- S57 200 543
- JP-A- S60 204 864
- JP-A- 2007 126 715
- JP-A- 2007 126 715
- JP-A- 2016 084 529
- JP-A- 2016 196 703
- JP-A- 2016 196 703
- JP-A- 2017 071 817
- JP-A- 2017 071 817
- US-A- 5 833 919

## Description

### TECHNICAL FIELD

This invention relates to high-Mn steel that is suitable for structural steel used in an extremely low-temperature environment such as a storage tank of liquefied gas, in particular, high-Mn steel excellent in toughness at low temperature, and a production method therefor.

JP 2016 196 703 A relates to a high Mn steel material for cryogenic use, wherein the volume fraction of austenite is 95% or more, the austenite has a crystal grain size of 20 to 200µm, and the carbide coverage ratio at the crystal grain boundary of the austenite is 50% or less.

### BACKGROUND

To use a hot-rolled steel plate in a structure for a storage tank of liquefied gas, the steel plate needs to have high strength and excellent toughness at low temperature because the structure is used at extremely low temperature. For example, when a hot-rolled steel plate is used for a storage tank of liquefied natural gas, excellent toughness needs to be guaranteed at the boiling point of the liquefied natural gas, that is, -164 °C or lower. When a steel material has poor low-temperature toughness, the safety as a structure for an extremely low temperature storage tank may not be maintained. Thus, there is a growing demand for steel materials with improved low-temperature toughness that are applied to such a structure. Hereinafter, an extremely low temperature range including -164 °C is referred to as "low temperature".

In view of the demand, austenitic stainless steel which has austenite as a microstructure of a steel plate, the austenite having no brittleness at low temperature, 9 % Ni steel, or five thousand series aluminum alloys have been conventionally used. However, the alloy cost and production cost are high, and thus there is a demand for steel materials which are inexpensive and excellent in low-temperature toughness.

As new steel materials replacing conventional steel for low temperature use, for example, JP 2017-71817 A (PTL 1) proposes using, as structural steel used in a low temperature environment, high-Mn steel added with a large amount of Mn which is a relatively inexpensive austenite-stabilizing element.

PTL 1 proposes a technique of controlling the Mn segregation ratio to prevent carbides generated in crystal grain boundaries from becoming an origin of fracture.

### CITATION LIST

### Patent Literature

PTL1: JP2017-71817A

### SUMMARY

### (Technical Problem)

Though it is possible to provide high-Mn steel excellent in low-temperature toughness according to the technique of PTL 1, there has been a demand for material cost reduction since the high-Mn steel needs to contain Ni from the viewpoint of guaranteeing toughness. Further, to reduce the Mn segregation ratio, diffusion heat treatment having a product of heating temperature (°C) and heating time (hr) of 30000 °C·hr or more is required, which incurs a high production cost.

It could thus be helpful to provide high-Mn steel excellent in low-temperature toughness which can suppress costs of materials and production. Further, it could be helpful to propose an advantageous method for producing such high-Mn steel. As used herein, the phrase "excellent in low-temperature toughness" means that the absorbed energy vE₋₁₉₆ in a Charpy impact test at -196 °C is 100 J or more.

### (Solution to Problem)

To achieve the aforementioned objects, the inventors conducted extensive study on high-Mn steel as to various factors determining the chemical composition and microstructure of a steel plate to discover the following:
a. Since high-Mn austenite steel has slow diffusion of Mn, a Mn segregation portion having a low Mn concentration formed during continuous casting remains after hot rolling. When the Mn segregation portion has a Mn concentration of less than 16 %, deformation-induced martensite forms at low temperature, deteriorating low-temperature toughness. Therefore, to improve the low-temperature toughness of high-Mn steel, it is effective to increase the Mn concentration in the Mn segregation portion.
b. Since high-Mn austenite steel has slow diffusion of Mn, a Mn segregation portion having a high Mn concentration formed during continuous casting remains after hot rolling. The Mn segregation having a Mn concentration of more than 38 % causes intergranular fracture, deteriorating low-temperature toughness. Therefore, to improve the low-temperature toughness of high-Mn steel, it is effective to decrease the Mn concentration in the Mn segregation portion.
c. With hot rolling under suitable conditions, the above a or b can be realized without diffusion heat treatment, and production costs can be suppressed.
d. Performing hot rolling under suitable conditions to provide a high dislocation density is effective for increasing yield stress.

The invention is conducted as described in claims 1 to 3.

Further, the KAM (Kernel Average Misorientation) value represents an average of orientation difference between each pixel (having a pitch of 0.3 µm) and the adjacent pixel in a crystal grain. For a steel plate after hot rolling, EBSD (Electron Backscatter Diffraction) analysis in a field of 500 µm × 200 µm was performed in arbitrary two fields, and an average of the analysis results for all the measured regions was calculated to determine an average KAM value.

### (Advantageous Effect)

According to this invention, it is possible to provide high-Mn steel excellent in low-temperature toughness. Therefore, our high-Mn steel largely contributes to the improvement of the safety and the service life of a steel structure used in a low temperature environment such as a tank for a storage tank of liquefied gas, and has industrially significant effects. Further, our production method does not decrease productivity or increase the production cost, and thus is excellent in economic efficiency.

### BRIEF DESCRIPTION OF THE DRAWINGS

In the accompanying drawings:
FIG. 1 is a graph representing a relationship between the Mn concentration of a negative Mn segregation portion and a Charpy absorbed energy (vE₋₁₉₆); and
FIG. 2 is a graph representing a relationship between the Mn concentration of a Mn segregation portion and a Charpy absorbed energy (vE₋₁₉₆).

### DETAILED DESCRIPTION

Our high-Mn steel will be described in detail hereinafter.

### [Chemical Composition]

The chemical composition of our high-Mn steel and the reasons for the limitations thereof are described first. In the description of the chemical composition, "%" denotes "mass%" unless otherwise noted.

### C: 0.100 % or more and 0.700 % or less

C is an inexpensive austenite-stabilizing element, and an important element to obtain austenite. To obtain this effect, the C content needs to be 0.100 % or more. On the other hand, a C content beyond 0.700 % generates excessive Cr carbides, deteriorating low-temperature toughness. Therefore, the C content is set to be 0.100 % or more and 0.700 % or less. The C content is preferably 0.200 % or more and 0.600 % or less.

### Si: 0.05 % or more and 1.00 % or less

Si acts as a deoxidizer, is necessary for steelmaking, and is effective at increasing the strength of a steel plate by solid solution strengthening when dissolved in steel. To obtain such an effect, the Si content needs to be 0.05 % or more. On the other hand, a Si content beyond 1.00 % deteriorates weldability. Therefore, the Si content is set to 0.05 % or more and 1.00 % or less, and preferably 0.07 % or more and 0.50 % or less.

### Mn: 20.0 % or more and 35.0 % or less

Mn is a relatively inexpensive austenite-stabilizing element. In this disclosure, Mn is an important element for achieving both strength and low-temperature toughness. To obtain the effects, the Mn content needs to be 20.0 % or more. On the other hand, a Mn content beyond 35.0 % deteriorates low-temperature toughness. Further, such a high Mn content deteriorates weldability and cuttability, and further promotes segregation as well as the occurrence of stress corrosion cracking. Therefore, the Mn content is set to 20.0 % or more and 35.0 % or less, preferably 23.0 % or more and 30.0 % or less, and more preferably 28.0 % or less.

### P: 0.030 % or less

When a P content is beyond 0.030 %, P segregates to grain boundaries and becomes an origin of stress corrosion cracking. Therefore, the upper limit of the P content is 0.030 %, and desirably, the P content is kept as small as possible. Therefore, the P content is set to 0.030 % or less. Excessively reducing P involves high refining cost and is economically disadvantageous. Therefore, the P content is desirably set to 0.002 % or more, preferably 0.005 % or more and 0.028 % or less, and more preferably 0.024 % or less.

### S: 0.0070 % or less

S deteriorates the low-temperature toughness and ductility of the base metal. Therefore, the upper limit of the S content is 0.0070 %, and desirably, the S content is kept as small as possible. Therefore, the S content is set to 0.0070 % or less. Excessively reducing S involves high refining cost and is economically disadvantageous. Therefore, the lower limit of the S content is desirably set to 0.001 % or more. The S content is preferably set to 0.0020 % or more and 0.0060 % or less.

### Al: 0.01 % or more and 0.07 % or less

Al acts as a deoxidizer and is used most commonly in molten steel deoxidizing processes to obtain a steel plate. To obtain such an effect, the Al content needs to be 0.01 % or more. On the other hand, when the Al content is beyond 0.07 %, Al is mixed into a weld metal portion during welding, deteriorating the toughness of the weld metal. Therefore, the Al content is set to 0.07 % or less. Therefore, the Al content is set to 0.01 % or more and 0.07 % or less, and preferably 0.02 % or more and 0.06 % or less.

### Cr: 0.5 % or more and 7.0 % or less

Cr is an element which stabilizes austenite with an appropriate amount of addition and is effective for improving low-temperature toughness and base metal strength. To obtain such effects, the Cr content needs to be 0.5 % or more. On the other hand, a Cr content beyond 7.0 % generates Cr carbides, deteriorating low-temperature toughness and stress corrosion cracking resistance. Therefore, the Cr content is set to 0.5 % or more and 7.0 % or less, preferably 1.0 % or more and 6.7 % or less, and more preferably 1.2 % or more and 6.5 % or less. To further improve stress corrosion cracking resistance, the Cr content is further preferably 2.0 % or more and 6.0 % or less.

### N: 0.0050 % or more and 0.0500 % or less

N is an austenite-stabilizing element and an element which is effective for improving low-temperature toughness. To obtain such an effect, the N content needs to be 0.0050 % or more. On the other hand, the N content beyond 0.0500 % coarsens nitrides or carbonitrides, deteriorating toughness. Therefore, the N content is set to 0.0050 % or more and 0.0500 % or less, and preferably 0.0060 % or more and 0.0400 % or less.

### O: 0.0050 % or less

O deteriorates low-temperature toughness because of the formation of oxides. Therefore, the O content is set to 0.0050 % or less, and preferably 0.0045 % or less. Excessively reducing O involves high refining cost and is economically disadvantageous. Therefore, the O content is desirably set to 0.0010 % or more.

### Ti: 0.005 % or less, and Nb: 0.005 % or less

Ti and Nb form carbonitrides with a high melting point in steel to prevent coarsening of crystal grains, then becoming an origin of fracture and a propagation path of cracks. In particular, in high-Mn steel, Ti and Nb hinder microstructure control for enhancing low-temperature toughness and improving ductility, and thus, need to be intentionally limited. Specifically, Ti and Nb are components which are inevitably mixed from raw materials and the like into steel, and Ti of more than 0.005 % and 0.010 % or less and Nb of more than 0.005 % and 0.010 % or less are typically mixed. Thus, according to the method described below, it is necessary to avoid inevitable mixing of Ti and Nb and limit the content of each Ti and Nb to 0.005 % or less. By limiting the content of each Ti and Nb to 0.005 % or less, it is possible to eliminate the adverse effect of carbonitrides and guarantee excellent low-temperature toughness and ductility. The content of each Ti and Nb is preferably set to 0.003 % or less. The contents of each Ti and Nb may be 0 %.

The balance other than the aforementioned components is Fe and inevitable impurities. The inevitable impurities include H, and a total content of 0.01 % or less is allowable.

### [Microstructure]

### Microstructure having austenite as a matrix phase

When a steel material has a body centered cubic (bcc) crystal structure, the steel material may cause brittle fracture in a low temperature environment, and thus, is not suitable for use in a low temperature environment. When the steel material is assumed to be used in a low temperature environment, the steel material is required to have, as a matrix phase, an austenite microstructure which has a face centered cubic (fcc) crystal structure. As used herein, the phrase "having austenite as a matrix phase" and similar phrases mean that the area ratio of an austenite phase is 90 % or more. The balance other than the austenite phase is a ferrite or martensite phase. The area ratio of the austenite phase is preferably 95 % or more.

As stated above, in high-Mn steel containing Mn in an amount of 20.0 % or more and 35.0 % or less, a segregation portion having a low Mn concentration and a segregation portion having a high Mn concentration, compared with the Mn content in the chemical composition are formed. As described below, the inventors found that these portions having different Mn concentrations are a factor behind the deterioration of low-temperature toughness.

Specifically, the Mn concentration of a Mn segregation portion and an absorbed energy in a Charpy impact test at -196 °C were measured on a steel plate obtained by hot rolling a steel material having the aforementioned chemical composition under various conditions. As used herein, the Mn segregation portion, which is a region having a low or high Mn concentration within a Mn segregation band, is specifically represented by a region having a lowest or highest Mn concentration which is measured by EBSD (Electron Backscatter Diffraction) analysis on a polished surface in a cross section along a rolling direction of a steel plate after hot rolling.

### Microstructure having Mn segregation portion with Mn concentration of 16 % or more and 38 % or less

First, in a Mn segregation portion having a low Mn concentration (negative Mn segregation portion), as FIG. 1 illustrates the result of measuring the Mn concentration and the absorbed energy in the Charpy impact test at -196 °C, it is found that when the Mn concentration in the Mn segregation portion is 16 % or more, an absorbed energy of 100 J or more is achieved. The Mn concentration in the Mn segregation portion is preferably 17 % or more.

Further, in a Mn segregation portion having a high Mn concentration, as FIG. 2 illustrates a result obtained by measuring the Mn concentration and the absorbed energy in the Charpy impact test at -196 °C, it is found that when the Mn concentration in the Mn segregation portion is 38 % or less, an absorbed energy of 100 J or more is achieved. The Mn concentration in the Mn segregation portion is preferably 37 % or less.

### Average KAM (Kernel Average Misorientation) value being 0.3 or more

As stated above, the KAM value is determined by performing EBSD (Electron Backscatter Diffraction) analysis in a field of 500 µm × 200 µm in an arbitrary two fields of a steel plate after hot rolling and calculating from the analysis results an average of orientation difference between each pixel (having a pitch of 0.3 µm) and the adjacent pixel in a crystal grain. The KAM value reflects the local crystal orientation change caused by dislocation in the microstructure. A higher KAM value represents a larger orientation difference between a measurement point and the adjacent portion. Specifically, a higher KAM value means a higher local deformation degree in a grain. Therefore, a higher KAM value in a steel plate after rolling means a higher dislocation density. Further, when the average KAM value is 0.3 or more, it means accumulation of a large amount of dislocation, and thus, yield stress increases. The average KAM value is preferably 0.5 or more. On the other hand, when the average KAM value is beyond 1.3, toughness may be deteriorated. Thus, the average KAM value is preferably 1.3 or less.

A Mn segregation portion having a Mn concentration of 16 % or more and 38 % or less and an average KAM value of 0.3 or more as stated above can be obtained by adjusting the chemical composition as described above and performing hot rolling according to the following conditions.

In this invention, to further improve strength and low-temperature toughness, in addition to the above essential elements, the following elements can be contained as necessary.

At least one of Mo: 2.0 % or less, V: 2.0 % or less, W: 2.0 % or less, Ca: 0.0005 % or more and 0.0050 % or less, Mg: 0.0005 % or more and 0.0050 % or less, and REM: 0.0010 % or more and 0.0200 % or less.
Mo, V, and W: 2.0 % or less

Mo, V, and W contribute to stabilizing austenite and improving base metal strength. To obtain such an effect, Mo, V, and/or W is preferably contained in an amount of 0.001 % or more. On the other hand, when the content of Mo, V, and/or W is beyond 2.0 %, coarse carbonitrides are generated, which may become an origin of fracture, and additionally increase production cost. Therefore, when Mo, V, and/or W is contained, the content of each added alloying element is 2.0 %, preferably 0.003 % or more and 1.7 % or less, and more preferably 1.5 % or less.

### Ca: 0.0005 % or more and 0.0050 % or less, Mg: 0.0005 % or more and 0.0050 % or less, REM: 0.0010 % or more and 0.0200 % or less

Ca, Mg, and REM are elements useful for morphological control of inclusions and can be contained as necessary. The morphological control of inclusions means granulating elongated sulfide-based inclusions. The morphological control of inclusions improves ductility, toughness, and sulfide stress corrosion cracking resistance. To obtain such effects, Ca and/or Mg is preferably contained in an amount of 0.0005 % or more and REM is preferably contained in an amount of 0.0010 % or more. On the other hand, when these elements are contained in a large amount, not only the amount of nonmetallic inclusions may be increased, ending up deteriorating ductility, toughness, and sulfide stress corrosion cracking resistance, but also an economic disadvantage may be entailed.

Therefore, when Ca and Mg are contained, the content of each element is set to 0.0005 % or more and 0.0050 % or less. When REM is contained, the content is set to 0.0010 % or more and 0.0200 % or less. Preferably, the Ca content is set to 0.0010 % or more and 0.0040 % or less, the Mg content is set to 0.0010 % or more and 0.0040 % or less, and the REM content is set to 0.0020 % or more and 0.0150 % or less.

Our high-Mn steel can be obtained from molten steel having the aforementioned chemical composition which is prepared by steelmaking using a publicly-known method such as using a converter and an electric heating furnace. In addition, the high-Mn steel may also be subjected to secondary refinement in a vacuum degassing furnace. During the secondary refinement, to limit the contents of Ti and Nb which hinder suitable microstructure control within the aforementioned range, it is necessary to prevent Ti and Nb from being inevitably mixed from raw materials or the like into steel and decrease the contents of Ti and Nb. For example, by decreasing the basicity of slag in the refining stage such that these alloy elements are concentrated in the slag to be discharged, it is possible to reduce the Ti and Nb concentrations in a final slab product. It is also possible to apply a method in which oxygen is blown into the furnace or the like for oxidation such that an alloy of Ti and Nb can be floated and separated during circulation. Subsequently, it is preferable to make the steel into a steel material such as a slab having a predetermined size by a publicly-known steel making method such as continuous casting.

The following provides a further definition of production conditions to make the aforementioned steel material into a steel material exhibiting excellent low-temperature toughness.

### [Heating temperature of steel material: 1100 °C or higher and 1300 °C or lower]

To obtain high-Mn steel having the aforementioned features, it is important to perform heating to a temperature range of 1100 °C to 1300 °C and hot rolling with a rolling finish temperature of 800 °C or higher and a total rolling reduction of 20 % or more. The temperature is controlled based on the surface temperature of the steel material.

Specifically, to promote diffusion of Mn during the hot rolling, the heating temperature before the rolling is set to 1100 °C or higher. On the other hand, a heating temperature beyond 1300 °C may trigger steel melting, and thus, the upper limit of the heating temperature is set to 1300 °C. The heating temperature is preferably 1150 °C or higher and 1250 °C or lower.

### [Rolling finish temperature of 800 °C or higher and total rolling reduction of 20 % or more]

Further, it is important to set the total rolling reduction during the rolling to as high as 20 % or more to thereby decrease the distance between Mn segregation portions such that diffusion of Mn is promoted. Similarly, from the viewpoint of promoting diffusion of Mn during the rolling, the rolling finish temperature is set to 800 °C or higher. This is because Mn is not sufficiently diffused at a temperature of lower than 800 °C, which is well below two thirds of the melting point of Mn. The rolling finish temperature is preferably 950 °C or higher and more preferably 1000 °C or higher and 1050 °C or lower. Further, the total rolling reduction is preferably 30 % or more. No upper limit is placed on the total rolling reduction, but from the viewpoint of improving rolling efficiency, the upper limit is preferably 98 %.

Further, if necessary, it is advantageous for increasing the KAM value to additionally perform the second hot rolling which satisfies the following conditions after the above hot rolling. Here, when the finish temperature of the above first hot rolling is 1100 °C or higher, the second hot rolling may be continued as it is, whereas when the finish temperature is lower than 1100 °C, re-heating to 1100 °C or higher is performed. Again, a heating temperature beyond 1300 °C may trigger steel melting. Thus, the upper limit of the heating temperature is set to 1300 °C. The temperature is controlled based on the surface temperature of the steel material. The heating temperature is preferably 1150 °C or higher and 1250 °C or lower.

### [Rolling finish temperature: 700 °C or higher and lower than 950 °C]

The second hot rolling requires at least one pass of final finish rolling at 700 °C or higher and lower than 950 °C. Specifically, by performing at least one pass of rolling preferably with a rolling reduction of 10 % or more at lower than 950 °C, dislocations having being introduced during the first rolling are less likely to be recovered and easily remain, and thus, the KAM value can be increased. Further, crystal grains become excessively coarse in a finish temperature range of 950 °C or higher, and thus desired yield stress cannot be obtained. Therefore, it is preferable to perform at least one pass of final finish rolling at lower than 950 °C. The finish temperature is preferably 900 °C or lower and more preferably 850 °C or lower.

On the other hand, a finish temperature of lower than 700 °C deteriorates toughness, and thus, the finish temperature is set to 700 °C or higher, and preferably 750 °C or higher. The rolling reduction at lower than 950 °C is preferably 20 % or more and more preferably 50 % or more. However, rolling with a rolling reduction of beyond 95 % deteriorates toughness, and thus, a rolling reduction of 95 % or less is preferable.

### [Average cooling rate within a range of a temperature at or above (a rolling finish temperature - 100 °C) to a temperature ranging from 300 °C to 650 °C: 1.0 °C/s or more]

After the hot rolling, cooling is immediately performed. Gentle cooling of the steel plate after the hot rolling promotes formation of precipitates, thus deteriorating low-temperature toughness. Cooling the steel plate at a cooling rate of 1.0 °C/s or more can prevent formation of these precipitates. Further, excessive cooling distorts the steel plate, deteriorating productivity. In particular, for a steel material having a plate thickness of less than 10 mm, air cooling is preferable. Therefore, the upper limit of the cooling start temperature is set to 900 °C. For the aforementioned reasons, in the cooling after the hot rolling, on a surface of the steel plate, the average cooling rate within a range of a temperature at or above (a rolling finish temperature - 100 °C) to a temperature ranging from 300 °C to 650 °C is set to 1.0 °C/s or more. Note that the subsequent heating treatment is unnecessary because the Mn segregation portions in the as-rolled state are maintained within a narrow Mn concentration range.

### EXAMPLES

This invention will be described in further detail below by way of examples. Note that this invention is not limited to the following examples.

Steel slabs having the chemical compositions listed in Table 1 were made by a converter-ladle refining-continuous casting process. Next, the obtained steel slabs were subjected to blooming (the first hot rolling) and hot rolling (the second hot rolling) under conditions listed in Table 2 to obtain steel plates having a thickness of 10 mm to 30 mm. Tensile properties, toughness, and microstructure of the obtained steel plates were evaluated as described below.

### (1) Tensile properties

JIS NO. 5 tensile test pieces were collected from each steel plate. Then, the test pieces were subjected to a tensile test in conformity with JIS Z 2241 (1998) to investigate tensile properties. In this invention, when a test piece had a yield stress of 400 MPa or more and a tensile strength of 800 MPa or more, the corresponding steel plate was determined to have excellent tensile properties. Further, when a test piece had an elongation of 40 % or more, the corresponding steel plate was determined to have excellent ductility.

### (2) Low-temperature toughness

Charpy V-notch test pieces were collected from each steel plate having a plate thickness of more than 20 mm at a 1/4 position of the plate thickness or from each steel plate having a plate thickness of 20 mm or less at a 1/2 position of the plate thickness, in a direction parallel to the rolling direction in conformity with JIS Z 2242 (2005). Then, the test pieces were subjected to Charpy impact test in conformity with JIS Z 2242 (2005), where three test pieces were used for each steel plate, to determine absorbed energy at -196 °C and evaluate base metal toughness. In this invention, when the three test pieces had an average absorbed energy (vE₋₁₉₆) of 100 J or more, the corresponding steel plate was determined to have excellent base steel toughness. For steel plates having a plate thickness of less than 10 mm, Charpy V-notch test pieces having a sub-size of 5 mm were collected from each steel plate at a 1/2 position of the plate thickness, in a direction parallel to the rolling direction in conformity with JIS Z 2242 (2005). Then, the test pieces were subjected to Charpy impact test at -196 °C in conformity with JIS Z 2242 (2005), where three test pieces were used for each steel plate. When the three test pieces had an average absorbed energy (vE₋₁₉₆) of 67 J or more, the corresponding steel plate was determined to have excellent base steel toughness.

### Percent brittle fracture

After the Charpy impact test at -196 °C, SEM observation (at 500 magnifications in 10 fields) was performed to measure percent brittle fracture. When the test pieces had a percent brittle fracture of 0 %, the corresponding steel plate was determined to have excellent low-temperature toughness.

### (3) Microstructure evaluation

### KAM value

For each steel plate after the hot rolling, EBSD (Electron Backscatter Diffraction) analysis (measurement step: 0.3 µm) in a field of 500 µm × 200 µm was performed in arbitrary two fields (at a 1/4 position of the plate thickness or and 1/2 position of the plate thickness) on a polished surface in a cross section along the rolling direction of the steel plate and an average of the analysis results for all the measured regions was calculated to determine an average KAM value.

### Deformation-induced martensite

After the Charpy impact test, the test piece was polished stepwise for convenience of observation to its notch bottom. In the test piece, five fields with a size of 100 µm × 100 µm were observed by EBSD analysis (measurement step: 0.08 µm) to determine the presence/absence of deformation-induced martensite.

### Mn concentration

Further, at the above-described positions where the KAM values were measured by EBSD, EPMA (Electron Probe Micro Analyzer) analysis was further performed to determine Mn concentrations, and those portions having the lowest Mn concentration and the highest Mn concentration were defined as segregation portions.

The results of these measurements are listed in Table 3.

**Table 1**

| Steel No. | Chemical composition (mass%) | | | | | | | | | | | | | | | | | Remarks |
|---|---|---|---|---|---|---|---|---|---|---|---|---|---|---|---|---|---|---|
| | C | Si | Mn | P | S | Al | Cr | O | N | Nb | Ti | V | Mo | W | Ca | Mg | REM | |
| 1 | 0.150 | 0.82 | 29.4 | 0.025 | 0.0058 | 0.034 | 3.78 | 0.0034 | 0.0150 | 0.002 | 0.002 | - | - | - | - | - | - | Example |
| 2 | 0.654 | 0.12 | 20.8 | 0.018 | 0.0042 | 0.028 | 2.78 | 0.0027 | 0.0132 | 0.002 | 0.002 | - | - | - | - | - | - | Example |
| 3 | 0.432 | 0.26 | 22.9 | 0.016 | 0.0039 | 0.037 | 4.81 | 0.0019 | 0.0259 | 0.001 | 0.002 | 0.09 | - | - | - | - | - | Example |
| 4 | 0.332 | 0.78 | 21.3 | 0.020 | 0.0065 | 0.045 | 3.12 | 0.0033 | 0.0191 | 0.002 | 0.003 | - | 0.48 | - | - | - | - | Example |
| 5 | 0.294 | 0.77 | 28.1 | 0.027 | 0.0028 | 0.063 | 1.87 | 0.0036 | 0.0243 | 0.001 | 0.002 | - | - | 0.09 | - | - | - | Example |
| 6 | 0.465 | 0.63 | 27.1 | 0.017 | 0.0024 | 0.038 | 6.19 | 0.0046 | 0.0350 | 0.003 | 0.003 | - | - | - | 0.0016 | - | - | Example |
| 7 | 0.327 | 0.46 | 22.5 | 0.018 | 0.0043 | 0.056 | 2.43 | 0.0032 | 0.0245 | 0.002 | 0.002 | - | - | - | - | 0.003 | - | Example |
| 8 | 0.364 | 0.41 | 20.2 | 0.028 | 0.0029 | 0.029 | 1.12 | 0.0042 | 0.0078 | 0.004 | 0.001 | - | - | - | - | - | 0.0044 | Example |
| 9 | 0.288 | 0.19 | 24.3 | 0.023 | 0.0057 | 0.047 | 5.78 | 0.0038 | 0.0334 | 0.002 | 0.001 | - | - | - | - | - | - | Example |
| 10 | 0.587 | 0.32 | 25.2 | 0.021 | 0.0034 | 0.045 | 4.24 | 0.0041 | 0.0092 | 0.003 | 0.001 | - | - | - | - | - | - | Example |
| 11 | 0.912 | 0.41 | 27.5 | 0.020 | 0.0024 | 0.038 | 3.43 | 0.0022 | 0.0113 | 0.002 | 0.002 | - | - | - | - | - | - | Comparative Example |
| 12 | 0.571 | 0.03 | 25.4 | 0.017 | 0.0027 | 0.037 | 5.11 | 0.0029 | 0.0387 | 0.002 | 0.002 | - | - | - | - | - | - | Comparative Example |
| 13 | 0.135 | 0.48 | 17.6 | 0.026 | 0.0019 | 0.049 | 2.33 | 0.0047 | 0.0471 | 0.001 | 0.001 | - | - | - | - | - | - | Comparative Example |
| 14 | 0.172 | 0.44 | 26.3 | 0.042 | 0.0025 | 0.039 | 0.87 | 0.0039 | 0.0334 | 0.001 | 0.003 | - | - | - | - | - | - | Comparative Example |
| 15 | 0.299 | 0.25 | 28.7 | 0.021 | 0.0084 | 0.027 | 1.86 | 0.0021 | 0.0062 | 0.002 | 0.001 | - | - | - | - | - | - | Comparative Example |
| 16 | 0.554 | 0.11 | 21.4 | 0.019 | 0.0034 | 0.090 | 3.69 | 0.0034 | 0.0224 | 0.002 | 0.003 | - | - | - | - | - | - | Comparative Example |
| 17 | 0.291 | 0.26 | 27.4 | 0.013 | 0.0025 | 0.061 | 8.25 | 0.0042 | 0.0143 | 0.003 | 0.002 | - | - | - | - | - | - | Comparative Example |
| 18 | 0.425 | 0.13 | 21.9 | 0.022 | 0.0049 | 0.024 | 3.77 | 0.0082 | 0.0241 | 0.002 | 0.002 | - | - | - | - | - | - | Comparative Example |
| 19 | 0.356 | 0.43 | 25.7 | 0.023 | 0.0036 | 0.053 | 6.37 | 0.0031 | 0.0589 | 0.004 | 0.002 | - | - | - | - | - | - | Comparative Example |
| 20 | 0.095 | 0.29 | 28.1 | 0.025 | 0.0036 | 0.042 | 6.12 | 0.0023 | 0.0095 | 0.002 | 0.002 | - | - | - | - | - | - | Comparative Example |
| 21 | 0.633 | 1.04 | 23.3 | 0.019 | 0.0040 | 0.035 | 2.53 | 0.0037 | 0.0170 | 0.002 | 0.002 | - | - | - | - | - | - | Comparative Example |
| 22 | 0.540 | 0.35 | 21.6 | 0.027 | 0.0033 | 0.050 | 0.47 | 0.0028 | 0.0210 | 0.001 | 0.003 | - | - | - | - | - | - | Comparative Example |
| 23 | 0.451 | 0.26 | 20.8 | 0.029 | 0.0060 | 0.035 | 2.87 | 0.0038 | 0.0327 | 0.006 | 0.002 | - | - | - | - | - | - | Comparative Example |
| 24 | 0.624 | 0.51 | 24.0 | 0.025 | 0.0052 | 0.028 | 3.18 | 0.0032 | 0.0188 | 0.002 | 0.006 | - | - | - | - | - | - | Comparative Example |
| 25 | 0.236 | 0.64 | 34.5 | 0.022 | 0.0061 | 0.042 | 1.45 | 0.0031 | 0.0363 | 0.002 | 0.002 | - | - | - | - | - | - | Example |
| 26 | 0.119 | 0.86 | 35.7 | 0.027 | 0.0063 | 0.029 | 0.55 | 0.0044 | 0.0466 | 0.002 | 0.002 | - | - | - | - | - | - | Comparative Example |
| 27 | 0.671 | 0.75 | 21.3 | 0.020 | 0.0047 | 0.008 | 0.94 | 0.0095 | 0.0377 | 0.001 | 0.001 | - | - | - | - | - | - | Comparative Example |
| 28 | 0.312 | 0.32 | 33.5 | 0.023 | 0.0034 | 0.045 | 0.50 | 0.0026 | 0.0139 | 0.002 | 0.002 | - | - | - | - | - | - | Example |

**Table 2**

| Sample | Steel No. | | First rolling conditions | | | Second rolling conditions | | | | Remarks |
|---|---|---|---|---|---|---|---|---|---|---|
| | | Plate No. thickness | Slab heating temperature | Rolling finish temperature | Total rolling reduction | Re-heating temperature | Rolling finish temperature | Cooling start temperature | Cooling rate within a range of 300 °C to 650 °C | |
| | | (mm) | (°C) | (°C) | (%) | (°C) | (°C) | (°C) | (°C/s) | |
| 1 | 1 | 22 | 1130 | 921 | 32 | 1130 | 810 | 774 | 8 | Example |
| 2 | 2 | 25 | 1130 | 918 | 29 | 1130 | 823 | 787 | 9 | Example |
| 3 | 3 | 18 | 1100 | 887 | 36 | 1100 | 765 | 702 | 9 | Example |
| 4 | 4 | 20 | 1100 | 892 | 35 | 1100 | 796 | 734 | 8 | Example |
| 5 | 5 | 25 | 1150 | 939 | 43 | 1150 | 838 | 805 | 8 | Example |
| 6 | 6 | 15 | 1150 | 937 | 46 | 1150 | 811 | 741 | 12 | Example |
| 7 | 7 | 10 | 1180 | 946 | 51 | 1180 | 805 | 728 | 16 | Example |
| 8 | 8 | 10 | 1200 | 953 | 53 | 1200 | 763 | 671 | 10 | Example |
| 9 | 9 | 13 | 1160 | 941 | 30 | 1160 | 813 | 762 | 7 | Example |
| 10 | 10 | 28 | 1250 | 1034 | 26 | 1250 | 946 | 915 | 16 | Example |
| 11 | 1 | 30 | 1300 | 1102 | 20 | - | 803 | 770 | 14 | Example |
| 12 | 11 | 20 | 1250 | 1011 | 30 | 1250 | 871 | 836 | 6 | Comparative Example |
| 13 | 12 | 15 | 1250 | 1019 | 41 | 1250 | 855 | 817 | 11 | Comparative Example |
| 14 | 13 | 20 | 1120 | 919 | 42 | 1120 | 789 | 748 | 12 | Comparative Example |
| 15 | 14 | 25 | 1120 | 931 | 29 | 1120 | 802 | 770 | 7 | Comparative Example |
| 16 | 15 | 20 | 1170 | 955 | 38 | 1170 | 820 | 774 | 3 | Comparative Example |
| 17 | 16 | 10 | 1170 | 937 | 53 | 1170 | 786 | 735 | 5 | Comparative Example |
| 18 | 17 | 20 | 1150 | 917 | 43 | 1150 | 801 | 756 | 13 | Comparative Example |
| 19 | 18 | 18 | 1150 | 926 | 32 | 1150 | 790 | 746 | 8 | Comparative Example |
| 20 | 19 | 13 | 1130 | 903 | 45 | 1130 | 767 | 710 | 12 | Comparative Example |
| 21 | 20 | 20 | 1150 | 920 | 38 | 1150 | 828 | 771 | 10 | Comparative Example |
| 22 | 21 | 18 | 1150 | 914 | 39 | 1150 | 821 | 760 | 7 | Comparative Example |
| 23 | 22 | 25 | 1170 | 956 | 30 | 1170 | 837 | 794 | 12 | Comparative Example |
| 24 | 23 | 14 | 1190 | 958 | 48 | 1190 | 819 | 762 | 8 | Comparative Example |
| 25 | 24 | 17 | 1190 | 966 | 46 | 1190 | 830 | 788 | 10 | Comparative Example |
| 26 | 1 | 17 | 1130 | 897 | 39 | 1130 | 682 | 587 | 8 | Comparative Example |
| 27 | 2 | 23 | 1200 | 956 | 16 | 1200 | 873 | 831 | 12 | Comparative Example |
| 28 | 3 | 15 | 1200 | 961 | 23 | 1200 | 841 | 780 | 0.5 | Comparative Example |
| 29 | 4 | 15 | 1230 | 756 | 37 | 1230 | 823 | 768 | 7 | Comparative Example |
| 30 | 5 | 20 | 1230 | 975 | 31 | 1230 | 810 | 653 | 3 | Comparative Example |
| 31 | 6 | 15 | 1050 | 888 | 25 | 1150 | 876 | 830 | 6 | Comparative Example |
| 32 | 7 | 25 | 1150 | 930 | 36 | 1050 | 731 | 687 | 10 | Comparative Example |
| 33 | 8 | 30 | 1250 | 1025 | 55 | 1300 | 980 | 947 | 9 | Comparative Example |
| 34 | 9 | 30 | 1300 | 704 | 75 | - | - | 655 | 6 | Comparative Example |
| 35 | 25 | 15 | 1130 | 906 | 35 | 1130 | 763 | 694 | 7 | Example |
| 36 | 25 | 15 | 1130 | 933 | 18 | 1130 | 707 | 655 | 6 | Comparative Example |
| 37 | 26 | 20 | 1150 | 934 | 42 | 1150 | 795 | 752 | 8 | Comparative Example |
| 38 | 27 | 6 | 1200 | 920 | 31 | 1200 | 734 | air cooling | - | Comparative Example |
| 39 | 28 | 6 | 1250 | 963 | 44 | 1250 | 860 | air cooling | - | Example |
| 40 | 1 | 30 | 1300 | 808 | 60 | - | - | 765 | 13 | Example |

**Table 3**

| Sample No. | Steel No. | Microstructure | | | | Mechanical properties | | | | | Remarks |
|---|---|---|---|---|---|---|---|---|---|---|---|
| | | Average KAM value | Deformation nduced martensite | Mn concentration in Mn segregation portion (lowest) | Mn concentration in Mn segregation portion (highest) | Yield stress | Tensile strength | Total elongation | Absorbed energy at-196°C (vE_{-196°C}) | Brittleness fracture | |
| | | | | (mass%) | (mass%) | (MPa) | (MPa) | (%) | (J) | (%) | |
| 1 | 1 | 0.9 | absent | 25.1 | 33.7 | 409 | 845 | 66 | 107 | 0 | Example |
| 2 | 2 | 0.8 | absent | 17.0 | 24.7 | 506 | 913 | 50 | 105 | 0 | Example |
| 3 | 3 | 1.1 | absent | 20.6 | 25.0 | 426 | 952 | 65 | 124 | 0 | Example |
| 4 | 4 | 1.0 | absent | 17.9 | 24.6 | 408 | 821 | 68 | 110 | 0 | Example |
| 5 | 5 | 0.7 | absent | 24.5 | 31.8 | 418 | 808 | 61 | 117 | 0 | Example |
| 6 | 6 | 0.9 | absent | 23.5 | 30.7 | 4S4 | 911 | 65 | 138 | 0 | Example |
| 7 | 7 | 1.2 | absent | 18.8 | 25.8 | 421 | 943 | 63 | 115 | 0 | Example |
| 8 | 8 | 0.8 | absent | 16.0 | 24.6 | 438 | 1012 | 69 | 102 | 0 | Example |
| 9 | 9 | 0.9 | absent | 21.3 | 27.3 | 413 | 957 | 6S | 131 | 0 | Example |
| 10 | 10 | 0.3 | absent | 22.6 | 27.4 | 401 | 925 | 67 | 153 | 0 | Example |
| 11 | 1 | 1.0 | absent | 23.5 | 35.6 | 420 | 855 | 64 | 103 | 0 | Example |
| 12 | 11 | 0.5 | absent | 23.3 | 31.5 | 614 | 755 | 47 | 61 | 25 | Comparative Example |
| 13 | 12 | 0.7 | absent | 22.2 | 28.7 | 385 | 930 | 67 | 124 | 0 | Comparative Example |
| 14 | 13 | 1.0 | present | 13.9 | 21.8 | 406 | 924 | 71 | 47 | 30 | Comparative Example |
| 15 | 14 | 0.9 | absent | 21.5 | 31.1 | 411 | 971 | 62 | 67 | 21 | Comparative Example |
| 16 | 15 | 0.9 | absent | 25.3 | 32.5 | 421 | 875 | 53 | 76 | 14 | Comparative Example |
| 17 | 16 | 1.0 | absent | 18.2 | 24,6 | 495 | 975 | 61 | 93 | 11 | Comparative Example |
| 18 | 17 | 0.9 | absent | 23.6 | 31.0 | 436 | 850 | 51 | 50 | 38 | Comparative Example |
| 19 | 18 | 1.0 | absent | 17.5 | 26.4 | 468 | 891 | S3 | 81 | 13 | Comparative Example |
| 20 | 19 | 1.1 | absent | 21.3 | 30.4 | S14 | 840 | 47 | 73 | 14 | Comparative Example |
| 21 | 20 | 0.8 | absent | 24.7 | 31.4 | 370 | 785 | 68 | 127 | 0 | Comparative Example |
| 22 | 21 | 0.8 | absent | 20.5 | 26.1 | 577 | 775 | 50 | 64 | 23 | Comparative Example |
| 23 | 22 | 0.7 | absent | 17.9 | 25.3 | 481 | 893 | 62 | 75 | 15 | Comparative Example |
| 24 | 23 | 0.9 | absent | 17.1 | 24.3 | 4S0 | 936 | 55 | 89 | 12 | Comparative Example |
| 25 | 24 | 0.7 | absent | 21.1 | 27.3 | 514 | 940 | 51 | 96 | 11 | Comparative Example |
| 25 | 1 | 1.5 | absent | 25.5 | 33.1 | 503 | 865 | 45 | 56 | 28 | Comparative Example |
| 27 | 2 | 0.5 | present | 15,7 | 25,9 | 536 | 923 | 50 | 95 | 11 | Comparative Example |
| 28 | 3 | 0.7 | absent | 20.8 | 25.3 | 415 | 876 | 43 | 61 | 24 | Comparative Example |
| 29 | 4 | 0.8 | present | 15.1 | 27.5 | 412 | 931 | 53 | 74 | 15 | Comparative Example |
| 30 | 5 | 0.8 | absent | 24,1 | 31.9 | 407 | 770 | 41 | 46 | 40 | Comparative Example |
| 31 | 6 | 0.4 | present | 15.8 | 37.7 | 440 | 899 | 46 | 93 | 11 | Comparative Example |
| 32 | 7 | 1.4 | absent | 18,6 | 26,1 | 468 | 941 | S4 | 73 | 15 | Comparative Example |
| 33 | 8 | 0.2 | absent | 16.5 | 24.0 | 365 | 933 | 72 | 116 | 0 | Comparative Example |
| 34 | 9 | 1.4 | absent | 20,7 | 27,7 | 553 | 802 | 43 | 41 | 45 | Comparative Example |
| 35 | 25 | 1.1 | absent | 30.8 | 38.0 | 427 | 760 | S6 | 102 | 0 | Example |
| 36 | 25 | 1.1 | absent | 30.5 | 38.6 | 459 | 787 | 52 | 80 | 13 | Comparative Example |
| 37 | 26 | 0.9 | absent | 31.8 | 39.4 | 4S0 | 777 | 50 | 52 | 35 | Comparative Example |
| 38 | 27 | 1.3 | absent | 17,7 | 24,9 | 494 | 902 | 52 | 58* | 12 | Comparative Example |
| 39 | 28 | 0.7 | absent | 30.8 | 363 | 449 | 886 | 54 | 73* | 0 | Example |
| 40 | 1 | 1.0 | absent | 26.1 | 32.5 | 418 | 846 | 65 | 104 | 0 | Example |

| | | | | | | | | | | | |
|---|---|---|---|---|---|---|---|---|---|---|---|
| ^{∗}5 mm sub-size charpy | | | | | | | | | | | |

Our high-Mn steel samples were all confirmed to satisfy the aforementioned desired performance (a base metal yield stress of 400 MPa or more and an average absorbed energy (vE₋₁₉₆) of 100 J or more for low-temperature toughness). In contrast, the comparative examples out of the scope of this invention did not satisfy the aforementioned desired performance in terms of either or both of yield stress and low-temperature toughness.

## Claims

1. High-Mn steel comprising:
a chemical composition containing, in mass%,
C: 0.100 % or more and 0.700 % or less,
Si: 0.05 % or more and 1.00 % or less,
Mn: 20.0 % or more and 35.0 % or less,
P: 0.030 % or less,
S: 0.0070 % or less,
Al: 0.01 % or more and 0.07 % or less,
Cr: 0.5 % or more and 7.0 % or less,
N: 0.0050 % or more and 0.0500 % or less,
O: 0.0050 % or less,
Ti: 0.005 % or less, and
Nb: 0.005 % or less;
optionally at least one selected from the group consisting of
Mo: 2.0 % or less,
V: 2.0 % or less,
W: 2.0 % or less,
Ca: 0.0005 % or more and 0.0050 % or less,
Mg: 0.0005 % or more and 0.0050 % or less, and
REM: 0.0010 % or more and 0.0200 % or less;
with the balance being Fe and inevitable impurities; and
a microstructure having austenite as a matrix phase, wherein the area ratio of an austenite phase is 90 % or more, **wherein**
the microstructure has a Mn segregation portion with a Mn concentration of 16 % or more and 38 % or less, and
the high-Mn steel has an average Kernel Average Misorientation value of 0.3 or more, an absorbed energy in a Charpy impact test at -196 °C of 100 J or more, and a yield stress of 400 MPa or more, which are measured by the methods disclosed in the description.

2. A method for producing high-Mn steel, comprising:
heating a steel material having the chemical composition according to claim 1 to a temperature range of 1100 °C or higher and 1300 °C or lower; and
a hot rolling step, in which hot rolling the steel material with a rolling finish temperature of 800 °C or higher and a total rolling reduction of 20 % or more is performed.

3. The method for producing high-Mn steel according to claim 2, further comprising:
a second hot rolling step, in which hot rolling the steel material with a rolling finish temperature of 700 °C or higher and lower than 950 °C is performed; wherein after the second hot rolling step,
the steel material is subjected to a cooling treatment at an average cooling rate of 1.0 °C/s or more within a range of a temperature at or above, the rolling finish temperature -100°C, to a temperature ranging from 300 °C to 650 °C.

## Patentansprüche

1. Stahl mit hohem Mn-Gehalt, umfassend:,
eine chemische Zusammensetzung, die in Masse-% umfasst:
C: 0,100 % oder mehr und 0,700 % oder weniger,
Si: 0,05 % oder mehr und 1,00 % oder weniger,
Mn: 20,0 % oder mehr und 35,0 % oder weniger,
P: 0,030 % oder weniger,
S: 0,0070 % oder weniger,
AI: 0,01 % oder mehr und 0,07 % oder weniger,
Cr: 0,5 % oder mehr und 7,0 % oder weniger,
N: 0,0050 % oder mehr und 0,0500 % oder weniger,
O: 0,0050 % oder weniger,
Ti: 0,005 % oder weniger und
Nb: 0,005 % oder weniger,
gegebenenfalls mindestens ein Element, ausgewählt aus der Gruppe bestehend aus:
Mo: 2,0 % oder weniger,
V: 2,0 % oder weniger,
W: 2,0 % oder weniger,
Ca: 0,0005 % oder mehr und 0,0050 % oder weniger,
Mg: 0,0005 % oder mehr und 0,0050 % oder weniger, und
REM: 0,0010 % oder mehr und 0,0200 % oder weniger,
wobei der Rest Fe und unvermeidbare Verunreinigungen sind, und
eine Mikrostruktur mit Austenit als Matrixphase, wobei das Flächenverhältnis einer Austenitphase 90 % oder mehr beträgt, wobei
die Mikrostruktur einen Mn-Segregationsanteil mit einer Mn-Konzentration von 16 % oder mehr und 38 % oder weniger aufweist, und
der Stahl mit hohem Mn-Gehalt einen durchschnittlichen Wert der durchschnittlichen kernbasierten Missorientierung von 0,3 oder mehr aufweist,
eine absorbierte Energie in einem Charpy-Kerbschlagbiegeversuch bei -196 °C von 100 J oder mehr und eine Streckspannung von 400 MPa oder mehr, die nach den in der Beschreibung angegebenen Verfahren gemessen werden.

2. Verfahren zur Herstellung von Stahl mit hohem Mn-Gehalt, umfassend:
Erhitzen eines Stahlmaterials mit der chemischen Zusammensetzung gemäß Anspruch 1 auf einen Temperaturbereich von 1100 °C oder höher und 1300 °C oder niedriger und
einen Warmwalzschritt, bei dem das Warmwalzen des Stahlmaterials mit einer Fertigwalztemperatur von 800 °C oder höher und einer Gesamtwalzreduktion von 20 % oder mehr durchgeführt wird.

3. Verfahren zur Herstellung von Stahl mit hohem Mn-Gehalt gemäß Anspruch 2, das ferner umfasst:
einen zweiten Warmwalzschritt, bei dem das Warmwalzen des Stahlmaterials mit einer Fertigwalztemperatur von 700 °C oder mehr und weniger als 950 °C durchgeführt wird,
wobei nach dem zweiten Warmwalzschritt das Stahlmaterial einer Abkühlungsbehandlung mit einer durchschnittlichen Abkühlungsrate von 1,0 °C/s oder mehr in einem Bereich von einer Temperatur bei oder über der Walzendtemperatur -100 °C bis zu einer Temperatur im Bereich von 300 °C bis 650 °C unterzogen wird.

## Revendications

1. Acier à forte teneur en Mn comprenant :
une composition chimique contenant, en % en masse,
C : 0,100 % ou plus et 0,700 % ou moins,
Si : 0,05 % ou plus et 1,00 % ou moins,
Mn : 20,0 % ou plus et 35,0 % ou moins,
P : 0,030 % ou moins,
S : 0,0070 % ou moins,
Al : 0,01 % ou plus et 0,07 % ou moins,
Cr : 0,5 % ou plus et 7,0 % ou moins,
N : 0,0050 % ou plus et 0,0500 % ou moins,
O : 0,0050 % ou moins,
Ti : 0,005 % ou moins, et
Nb : 0,005 % ou moins ;
facultativement au moins l'un choisi dans le groupe constitué de
Mo : 2,0 % ou moins,
V : 2,0 % ou moins,
W : 2,0 % ou moins,
Ca : 0,0005 % ou plus et 0,0050 % ou moins,
Mg : 0,0005 % ou plus et 0,0050 % ou moins, et
REM : 0,0010 % ou plus et 0,0200 % ou moins ;
le reste étant constitué de Fe et d'impuretés inévitables ; et
une microstructure ayant de l'austénite comme phase de matrice, dans lequel le rapport de surface d'une phase austénite est de 90 % ou plus, dans lequel
la microstructure a une partie de ségrégation de Mn avec une concentration en Mn de 16 % ou plus et de 38 % ou moins, et
l'acier à forte teneur en Mn a une valeur moyenne de désorientation moyenne locale de 0,3 ou plus, une énergie absorbée lors d'un essai de choc Charpy à -196°C de 100 J ou plus, et une limite d'élasticité de 400 MPa ou plus, qui sont mesurées par les procédés décrits dans la description.

2. Procédé de production d'acier à forte teneur en Mn, comprenant :
le chauffage d'un matériau en acier ayant la composition chimique selon la revendication 1 jusqu'à une plage de température de 1 100°C ou plus et de 1 300°C ou moins; et
une étape de laminage à chaud, dans laquelle un laminage à chaud du matériau en acier avec une température de finition de laminage de 800°C ou plus et une réduction totale de laminage de 20 % ou plus est effectué.

3. Procédé de production d'acier à forte teneur en Mn selon la revendication 2, comprenant en outre :
une seconde étape de laminage à chaud, dans laquelle un laminage à chaud du matériau en acier avec une température de finition de laminage de 700°C ou plus et inférieure à 950°C est effectué ; dans lequel après la seconde étape de laminage à chaud,
le matériau en acier est soumis à un traitement de refroidissement à une vitesse de refroidissement moyenne de 1,0°C/s ou plus dans une plage de température égale ou supérieure à la température de finition de laminage - 100°C, jusqu'à une température dans la plage de 300°C à 650°C.
